

## UNITED STATES PATENT OFFICE

2,263,730

## METHOD FOR IMPROVING TEXTILE MATERIAL

Winfried Henrich, Dusseldorf-Reisholz, Richard Hueter, Dessau-Rossbau-in-Anhalt, and Heinz-Joachim Engelbrecht, Dessau-in-Anhalt, Germany, assignors, by mesne assignments, to Heberlein Patent Corporation, New York, N. Y., a corporation of New York

No Drawing. Application February 19, 1938, Serial No. 191,494. In Germany February 19, 1937

9 Claims. (Cl. 8—113)

It is known that textile fibres, fibre-materials or tissues can be refined or impregnated by exposing the same to the action of baths consisting of solutions of esters of iso-cyanic acid or, respectively, of iso-thio-cyanic acid containing higher molecular alkyl groups. The impregnations obtained in this way are fast to a slight washing with soap as well as to the action of fat-solvents such as benzine or the like.

Now it has been found that analogous effects are obtainable in a very easy and advantageous manner by impregnating the textile material with a carbodiimide compound containing at least one higher molecular aliphatic radical having no less than 10 carbon atoms.

The substances found valuable are carbodiimide compounds containing at least one higher molecular aliphatic radical having no less than 10 carbon atoms. The carbodiimide radical may be combined directly or through any suitable atoms or atomic groups with one or several higher molecular alkyl radicals.

It is of course not necessary that the alkyl radical be of a homogeneous nature. The alkyl radical will vary according to the nature of the commercially obtainable higher molecular alkylating agents, which in general are not quite homogeneous. We may also consider for the present method substances with alkyl substituents, of a different chain-length. The chain length varies according to the initial applied material.

Compared with the substances hitherto suggested and particularly with the esters of iso-cyanic acid and isothiocyanic acid the di-phenyl-carbodi-imides offer the advantage of being easily accessible. For instance it would be sufficient to treat with carbon disulfide and an aniline which may be alkylated in the nucleus ("alkyl" containing no less than 10 C atoms) and to separate hydrogen sulfide from the reaction product according to the well-known method by mercuric oxide, lead-carbonate or the like. The course of the reactions corresponds to the following equations:



Unsymmetrical mono-substituted diaryl-carbodi-imides are obtainable in the same way from the unsymmetrical thio-carbamides. The unsymmetrical thio-carbamides are produced according to the well-known method by the reaction of phenyl-mustard oil upon alkyl-substituted ani-

lines or the like. The course of reaction is quite smooth. In a similar way the phenyl-carbodi-imides are developed from phenyl-isocyanic acid esters by heating to higher temperatures. The action of the substances will not be impaired if the higher molecular alkyl residue is not substituted directly in the nucleus as it may be bound indirectly to the phenyl nucleus by means of another atom or another atom grouping. As an example there may be cited the substances obtainable from carbon disulfide and alkyl-ethers of the amido-phenols, which after the de-sulfurization with lead-carbonate result as high molecular alkoxy-phenyl-carbodi-imides. Those substances are applied preferably in indifferent solvents such as benzol, benzine, chlorinated hydrocarbons or the like.

In the further development of this invention it has also been found that the effect produced by the treatment of textiles with high molecular diaryl-carbodi-imide derivatives, can likewise be obtained with differently substituted carbodi-imides, provided they contain at least one alkyl-residue with no less than 10 C atoms. Thus for example, aryl-alkyl-carbodiimides are produced with one or several alkyl-substituents containing no less than 10 C atoms, which alkyl substituents may be bound on the aromatic nucleus as well as on the not otherwise substituted nitrogen atom. The higher molecular dialkyl-carbodiimides are also useful in the same above described sense. Derivatives of cyanamide may be designated by the formula  $HN=C=N.R$ , where R contains an alkyl residue of not less than ten carbon atoms. These substances may also be employed in our process as they are in fact carbodiimide derivatives.

The preparation of said substances is performed by well known methods, that is, by de-sulfurization of the corresponding thio-carbamides with lead-oxide, lead-carbonate or mercuric oxide. The reaction follows in most cases in a practically quantitative yield. Only the mere aliphatic thio-carbamides offer some difficulties in the de-sulfurizing according to this method, as a substitution of the sulfur atom by oxygen often takes place, so that carbamide-derivatives are simultaneously developed. The carbodiimides are applicable either after separating those indifferent by-products or mixed with such accompanying bodies.

## Example 1

1.4 kgs. of cetyl-aniline (containing octadecyl-aniline and obtained according to the method of

Krafft, "Ber. d. Dtsch. Chem. Ges. 19 page 2984") are heated with 5 kgs. of carbon disulfide and 0.016 kg. of sulfur-powder to a slight boiling until the development of hydrogen-sulfide ceases completely. While still warm the cetyl-phenyl-thio-carbamide forms crystals of the lamellar shape. After sucking off the liquid and drying the crystals 6 kgs. of toluol are brought in without previously cleaning the crystals. In order to convert into the di-(cetyl-phenyl)carbodiimide 1.4 kgs. of lead-carbonate are brought into the toluol-solution at 100° C. while being stirred. The stirring is continued at this temperature until a sample filtered off results after evaporating as a wax-like residue solid at room-temperature and free of sulfur. Then by filtration the leaf-sulfide is separated off. The thus obtained solution can be applied directly as mother-solution. For impregnating-purposes it is diluted with benzol, benzine or the like up to  $\frac{1}{2}$  to 1%.

With a solution diluted in the aforesaid manner light fibers are treated at room-temperature for approximately 10 minutes, and heavy fibers up to half an hour. Then they are squeezed out and dried at 80-100° C., whereupon one continues heating for 1 to 2 hours at 110-125° C. Fibers of artificial silk get particularly water-repellent by this treatment. The impregnation proved to be stable as neither a repeated washing with soap nor an extraction with benzine were able to neutralize the impregnating effect.

#### Example 2

1.2 kgs. of hexa-decyl-p-amidophenol ether, 4.5 kgs. of carbonic disulfide and 0.015 kg. of sulfur-powder are heated to a slight boiling until the development of hydrogen-sulfide ceases completely. After cooling one sucks off the remaining liquid and the deposit is washed out with spirit. The thus resulting hexa-decoxy-phenyl-thio-carbamide (boiling point 139.5° C.) in the form of colourless lamellar crystals is dissolved without further purification in 5 kgs. of toluol, and treated with an excess of lead-carbonate (1 kg.) at about 100° C. while being stirred for 30 to 40 minutes. The thus formed lead-sulfide is filtered off. The approximately 18-20% solution if evaporated leaves, at room temperature, a solid waxlike substance. Instead of evaporating it may be diluted for use with benzine or benzol to the desired proportion for use.

With a solution of the above product, diluted up to 1% of solid content, fibers of artificial silk were treated at 20° C. for 10 minutes, then dried at 100° C. and then left for one hour in the drying oven at 110-120°. After this treatment the fibers had an agreeable soft handle and were strongly water-repellent. After washing eight times in a cocoanut oil-soap bath containing 0.25% of fatty acid, no diminution of those properties could be observed.

Mixed fibers consisting of wool and cotton and treated in the same way became likewise strongly water-repellent. This impregnation also proved fast to washing with benzine.

#### Example 3

A mixture of 0.67 kg. of phenyl-mustard-oil and 1.6 kgs. of cetyl-p-amido-phenyl ether is dissolved in 6 kgs. of benzol and kept boiling under a reflux condenser for 2 hours. Then with mechanical stirring it is treated with lead-carbonate (about 2.8 kgs.) until a sample filtered off leaves

a residue free of sulfur, whereupon the mixture is filtered.

The effects obtained with a dilution of the filtrate containing 1% of solid substance, in treating viscose-silk, cotton materials or woolen fibers are, after drying and subsequent treatment at a temperature up to 120° C., in exact accordance with those described in Example 2.

#### Example 4

To produce a dilauryl-carbodiimide suitable for the purpose of the present invention we avail ourselves of monolauryl-amine (technical, boiling point 0.8 mm.: 96.5 to 97.5° C.). By treatment with carbon disulfide it changes over into lauryl-dithio-carbamide-acid lauryl-amine, which when heated up to 110-120° C. forms di-lauryl-thio-carbamide (boiling point, after re-crystallization from alcohol, 80.5°). This is now converted into dilauryl-carbodiimide by further treatment with an excess of ten times the weight of mercuric oxide at a temperature of 110-120° C. The isolation of the carbodiimide (yellowish oil slowly solidifying when kept at room temperature) is obtained by dissolving it in cold benzol from the reaction-mixture. For the impregnation we take a 0.5-1%-solution in benzol. The material is agitated in this solution for 10 minutes at 20-30° C., whereupon it is centrifuged and dried. By heating the material for 1 hour up to 110-120° the fixation of the impregnation will occur. This impregnation imparts to woolen cloths, mixed fibers and artificial silk materials the property of water-repelling to a surprisingly high degree. This impregnation proved fast to a mild soap-washing as well as to benzine-washing.

#### Example 5

A mixture of 2 kgs. of hexadecyl-p-amidophenol ether, 1 kg. of allyl-mustard oil and 4 kgs. of toluol are heated to 100° C. for 5 hours, whereupon the solvent is removed by distilling. After cooling the residue is stirred with ether and the liquid sucked off. The thus resulting hexadecoxy-allyl-thiocarbamide (boiling point 96.5°) in the form of light powder is treated in 5 kgs. of toluol with an excess of lead-carbonate under vigorous stirring and at a temperature of approximately 100° C. The thus formed lead-sulfide is filtered off and the solution is applicable for the impregnation after dilution to the desired degree.

Artificial silk-satin, treated for 10 minutes with a 1% solution diluted with benzine and then dried for 2 hours at temperatures gradually rising to 120° C., is of a soft handle. At the same time this impregnation eliminates the water absorptive power. Those effects could not be reduced even by washing several times in a 0.5%-solution of soap-flakes. The water repellent property remained after a washing with benzine.

#### Example 6

1 kg. of hexadecoxy-p-phenyl-mustard oil is dissolved in 5 kgs. of toluol and treated at 80° C. with dry ammonia-gas for about 2 hours. While cooling, the mono-hexadecoxy-p-phenyl-thiocarbamide forms crystals which are brilliant and colourless; these crystals are liberated from the solvent by sucking off the latter (boiling point 127° C.). The crystalline product is de-sulfurized with lead-carbonate in a toluol-solution (as per Example 2), whereupon it is separated from the lead-sulfide by filtration; then the solution is evaporated in a vacuum. There remains a wax-

like mass (mono-hexa-decoxy-p-phenyl-carbodiimide or hexa-decoxy-p-phenyl-cyanamide). The product is suitable for impregnating wool, cotton, mixed tissues and the like to render them water repellent. An artificial silk-satin impregnated for 10 minutes with a 0.5-1%-solution in benzol and subsequently treated (as per Example 2) has a very remarkable water-repelling power which is fast to washing. In a similar way materials of wool or mixed fibers can be impregnated to become water-repellent.

*Example 7*

A mixture of 1 kg. of N-octadecyl-chloro-acetamide (boiling point 78° C.), is produced by converting octadecyl-amine with an equi-molecular amount of chloro-acetyl-chloride in the presence of pyridine, and 0.2 kg. of the mono-sodium-salt of cyanamide, such mixture is heated up to 120-130° with vigorous stirring of 7 kgs. of dibutyl ether and a small amount of copper-bronze powder. After removal of sodium-chloride one filters off from the precipitated salt and the solvent distilled off. The thus obtained residue is a wax-like mass solid at room-temperature and is easily soluble in organic solvents such as benzine, benzol etc. This mass dissolved in benzol is suitable for treatment of fibers in a manner similar to that of the preceding examples for providing water-repellence.

We claim:

1. The method for improving textile material characterized by impregnating the textile material by a carbodiimide compound containing at least one higher molecular alkyl radical having at least 10 carbon atoms, and heating the impregnated material at temperatures above 100° C. to produce a reaction by the said compound to produce water-repellency in the fibre.

2. The method for improving textile material characterized by impregnating the textile material by a carbodiimide compound containing at least one higher molecular hydrocarbon radical of the group consisting of alkyl, aralkyl, alkylaryl radicals having at least 10 carbon atoms in the alkyl portion thereof, and heating the impregnated material at a temperature between 105-120° C. to produce a reaction by the said compound to produce water-repellency in the fibre.

3. The method for improving textile material characterized by impregnating the textile material by a carbodiimide compound containing at

least one higher molecular alkyl radical having at least 10 carbon atoms, having at least one heteroatom in the aliphatic chain and heating the impregnated material to produce a reaction by the said compound to produce water-repellency in the fibre.

4. The method for improving textile material characterized by impregnating the textile material by a carbodiimide compound containing at least one higher molecular aliphatic radical having no less than 10 carbon atoms and heating the impregnated material to produce a reaction by the said compound to produce water-repellency in the fibre.

5. The method for improving textile material characterized by impregnating the textile material by a diarylcarbodiimide having at least one alkyl radical in the compound containing no less than 10 carbon atoms and heating the impregnated material to produce a reaction by the said compound to produce water-repellency in the fibre.

6. The method for improving textile material characterized by impregnating the textile material by a carbodiimide compound containing an alkyl-aryl radical having an oxygen atom in the hydrocarbon chain and at least 10 carbon atoms therein, and heating the impregnated material to produce a reaction by the said compound to produce water-repellency in the fibre.

7. The method for improving textile material characterized by impregnating the textile material by a carbodiimide compound containing an aliphatic radical having an —NH—CO— group in the hydrocarbon chain and at least 10 carbon atoms therein, and heating the impregnated material to produce water-repellency in said textile material.

8. A textile treating agent for imparting water-repelling properties to textiles which consists in a carbodiimide compound having at least one higher molecular aliphatic radical containing no less than 10 carbon atoms.

9. A textile treating agent for imparting water-repelling properties to textiles which consists in a carbodiimide having two aryl radicals and at least one alkyl radical containing no less than 10 carbon atoms.

50

WINFRID HENTRICH.  
RICHARD HUETER.  
HEINZ-JOACHIM ENGELBRECHT.

CERTIFICATE OF CORRECTION.

Patent No. 2,263,730.

November 25, 1941.

WINFRID HENTRICH, ET AL.

It is hereby certified that error appears in the printed specification of the above numbered patent requiring correction as follows: Page 1, first column, line 31, for the words "applied material" read --material applied--; line 50, for "diaryl-varbodi-" read -- diaryl-carbodi- --; page 2, first column, line 17, for "leaf-sulfide" read --lead-sulfide--; page 3, first column, line 20, after "stirring" insert --, in the presence--; line 23, after "solvent" insert --is--; and that the said Letters Patent should be read with this correction therein that the same may conform to the record of the case in the Patent Office.

Signed and sealed this 15th day of January, A. D. 1942.

(Seal)

Henry Van Arsdale,

Acting Commissioner of Patents.